

Feb. 16, 1932.

J. B. WELLS

1,845,377

PROCESS OF MAKING NITROCELLULOSE FILMS AND SIMILAR PRODUCTS

Original Filed Feb. 10, 1928



*Inventor,*  
Jackson B. Wells,

*By R. L. Stinchfield*

*Attorney*

## UNITED STATES PATENT OFFICE

JACKSON B. WELLS, OF ROCHESTER, NEW YORK, ASSIGNOR TO EASTMAN KODAK COMPANY, OF ROCHESTER, NEW YORK, A CORPORATION OF NEW YORK

## PROCESS OF MAKING NITROCELLULOSE FILMS AND SIMILAR PRODUCTS

Application filed February 10, 1928, Serial No. 253,361. Renewed March 9, 1931.

This invention relates to processes of making nitrocellulose films and similar products,—especially processes in which the films are set by liquid baths instead of by evaporation. One object of the invention is to provide an inexpensive process of this nature which will produce flexible, transparent, nitrocellulose films, filaments, etc., rapidly with minimum fire-risk and with maximum recovery of the solvents employed. Another object is to provide a process of this nature which can be carried out in a relatively small and simple apparatus. A still further object is to provide a process in which cloudiness in the films is avoided in spite of the use of rapid or aqueous setting baths. Other objects will hereinafter appear.

In the accompanying drawing the single figure is a diagrammatic side elevation, with the top broken away, of one form of apparatus in which my process may be carried out, the relative sizes of the parts being exaggerated for the sake of clearness.

I have found that the desired objects can be attained by shaping into film or filament form a nitrocellulose solution or "dope" containing methyl alcohol and a monohydroxy aliphatic alcohol of low volatility which is at least partially soluble in water, and setting it, while in this form, by treatment with an aqueous bath. While plain cold water may be used, I prefer to employ a setting bath in which there is a nitrocellulose solvent, miscible with water but of insufficient amount to prevent the setting action, said solvent regulating the setting operation. For example, a bath of water and methyl alcohol has proven to be very useful.

The presence of an alcohol of low volatility in the dope, such as normal butyl alcohol for instance, has been found to be of special benefit, during the setting step, because it lessens the danger of forming whitish or clouded defects in the film. In fact, typical rapid film-setting conditions, which have produced clouded products from plain nitrocellulose-methyl alcohol dopes, have been found to produce clear transparent films when applied to similar dopes containing a higher alcohol. This tendency of the higher

alcohols toward the formation of transparent films permits wider tolerances in the conditions of film-setting and allows higher speed of production without harm.

It is a fortunate advantage of my film-forming operation that it fits in both with preceding and subsequent steps. For example, considerable dehydration of washed nitrocellulose fibers must be accomplished before a film dope can be made from them. 55 The use of normal butyl alcohol for this purpose is disclosed in U. S. Patent No. 1,398,911, Seel, November 29, 1921. It forms a mass of nitrocellulose fibers containing about 40 to 60% of butyl alcohol. This, when dissolved 60 in methyl alcohol, as described in U. S. Patent No. 1,380,258, Seel, Combs, and Kemp, May 31, 1921, produces a dope having the desirable properties for making film by my present process. After the films are formed, 65 they are coated to form photographic films; and the continued presence of a higher alcohol, such as butyl alcohol, in such films promotes better wearing qualities and increased 70 flexibility, as described in said last-named 75 patent. It will, therefore, be seen that the higher alcohol passes successfully from the dehydration through my film-forming operation to the finished films, and is a beneficial ingredient—not a passive diluent—during 80 such operation.

I shall now describe one way of carrying out my process, by way of illustration, but it will be understood that the invention is not limited to the details thus given, except 85 as indicated in the appended claims. 100 parts by weight of cellulose nitrate fibers, of the type usually made up into film, are dehydrated with butyl alcohol and pressed until they contain from 30 to 100, say 50, parts 90 by weight of butyl alcohol in the mass, as indicated in the hereinabove cited patents. This mass is then dissolved in 300 to 1000 parts by weight, say 500 parts, of methyl alcohol and the ingredients thoroughly stirred, 95 say in a mixing apparatus, until the solution is substantially homogeneous.

This viscous dope, after filtering, if necessary, is then loaded into the V-shaped trough 100 of the apparatus shown in the drawing.

The lower part of this trough is provided with accurate edge pieces 2, 3, the latter being regulated up and down by the screw 4, thereby regulating the thickness of the film 5 from dope 6. Edge piece 2 projects slightly below edge piece 3, thus guiding the accurately gauged film-shaped dope onto the accurately polished cylindrical surface 7 of wheel 8. This surface may be that shown in U. S. 10 Patent No. 1,466,733, Sulzer, September 4, 1923, but any other suitable surface, such as polished electro-deposited chromium, may also be used. The wheel 8 turns in the direction of the arrow, the sheet of dope on the 15 surface 7 passing through a chamber 9. In this chamber the film-shaped body 5 of dope is still in a slowly flowable condition and can, therefore, settle under the influence of gravity sufficiently to enable the thickness of the 20 layer to equalize. In other words, if portions of the layer are slightly too thick and other portions are slightly too thin, in spite of the accuracy of edge pieces 2 and 3, these 25 inequalities will gradually work out in chamber 9 by the settling of the higher portions and the raising of the lower portions.

The equalized film-form layer 5 is then carried by continued revolution of the wheel 8 into the setting bath 10. The latter can 30 be conveniently contained in a vessel which is substantially concentric with and spaced from the outer surface 7 of the wheel 8, as indicated in dotted lines in the drawing. While other forms may be used, this has the 35 advantage of enabling the liquids of the bath to enter by pipe 11 and pass in a direction counter to the movement of the film, finally leaving the apparatus through exit pipe 12. As the setting bath proceeds from pipe 11 to 40 pipe 12 in the direction of the arrows, it becomes more and more charged with methyl alcohol, which it extracts from the layer 5 on the surface 7. Conversely the layer 5 starts to set when it enters the bath adjacent 45 to the pipe 12 and gradually gives up more and more of its methyl alcohol to the bath as it proceeds toward the entrance pipe 11. In other words, the more firmly the film becomes set and the more it loses the methyl 50 alcohol, the stronger is the setting bath with which it contacts. Since the bath, when it leaves pipe 12, contains its maximum percentage of methyl alcohol, it is in the best condition for the recovery of the latter by 55 the usual processes, say by fractional distillation.

While I can introduce plain water through pipe 11 as the initial ingredient of the setting bath, and allow the latter to increase in 60 methyl alcohol content, as it extracts methyl alcohol, during its passage through the apparatus, I prefer to introduce through the pipe 11 a mixture of a non-solvent for the nitrocellulose, such as water, and a solvent 65 for it, such as methyl alcohol. A 50% aque-

ous solution by weight of methyl alcohol has proven to be very useful. This becomes stronger as it proceeds through the apparatus to the exit pipe 12, by reason of the extraction of methyl alcohol from layer 5, and 70 entrance of water into the film.

Of course, in any event there is some extraction of the higher alcohol, such as butyl alcohol, from the film, but there is always a substantial amount of it left in the film to maintain flexibility and wearing qualities in the latter. In fact, the rotation of the wheel 8, the rate of flow of the bath 10, the strength of the bath 10, and the length of the bathing chamber are always coordinated so as to leave 80 the film with a useful content of the higher alcohol, say of the order of 1 to 10% of the weight of nitrocellulose; but this may be considerably higher, say 20%, depending upon the extent of curing or drying after the set 85 film is stripped from the surface 7. It will thus be seen that there is considerable latitude in the content of butyl alcohol in a film which is strong enough to be stripped, but a useful residuum of this alcohol always remains. In fact, even a considerable amount of methyl alcohol may remain in the stripped film and be removed by subsequent drying or "curing" operations, such as heretofore used 90 on films formed by evaporation. Any higher alcohol which is taken up by the bath 10 can readily be recovered by fractional distillation and used again. Its presence in the bath does not interfere with the action of the latter.

Between the point where the set film 51 is stripped from the surface 7 and the point where the layer 5 of dope is deposited upon 7, there may be located any suitable cleaning or polishing apparatus, such, for instance, as 105 that described in U. S. Patent No. 1,187,929, Reid, June 20th, 1916. A pipe 15 is provided with fine perforations in its under side through which water is sprayed onto the surface 7. This pipe is parallel to the axis of 110 drum 8. The cleaning liquid is not allowed to flow down the surface 7 to the stripped film 51 or the bath 10, but is taken up by a dam in the shape of a hollow roll 16 having its periphery covered with a layer of soft rubber 115 17 through which a series of fine apertures are provided communicating with the interior of the roll, the latter being connected to a vacuum apparatus, thus sucking the water through the dam and out of the apparatus. The surface of the drum may be given a final 120 conditioning by an absorbent roll 19, held against the surface by an adjustable spring 20.

Since the inner side of the film, which is stripped from the surface 7, is kept from contact with liquids, and since the outer surface passes over smooth roll 13, and is squeegeed by the latter, the film 51 carries little or no surface liquid, and is in condition to be dried, 125 cured and coiled by the known methods here- 130

tofore used in the production of nitrocellulose films by evaporation.

The trough 1 may be kept above room temperature, if desired, to keep the dope 6 at the right viscosity for formation of the layer 5, and may be covered to prevent the loss of volatile solvents. Both of these expedients, being well known in the art are, for the sake of simplicity, omitted from the drawing. The 10 bath 10 may vary in temperature over a considerable range, although, in general, it is preferable to operate at lower temperatures, the higher the percentage of water in the bath 10. For example, if pure water be introduced through pipe 11, a temperature of about 4° C. is useful. But with baths containing 50% or more of methyl alcohol, there is no need for such low temperature. I usually prefer, however, to keep the entire apparatus, 15 with the exception of trough 1, at or below room temperature, say 23° C., because with higher temperatures the tendency towards cloudiness becomes greater.

My process may be applied to films of thicknesses customarily employed in the photographic art, but thicker ones, and even somewhat thinner ones, may be obtained in a state of satisfactory transparency, flexibility and strength. The setting action imparts sufficient strength to the film to allow it to be stripped from the surface 7; in fact, the setting action seems to counteract any harmful sticking tendency of the dope on the surface 7.

While I prefer to use normal butyl alcohol, because it is most readily available commercially, my process may be carried out with other monohydroxy aliphatic alcohols having a low volatility, such as isobutyl alcohol, and the different isomeric amyl alcohols, or mixtures of them, commonly available in fusel oil. It will be noted that these all have boiling points somewhat above that of water.

In the preferred form of my process the methyl alcohol used in the dope contains less than 1% of water and the dehydrated nitrocellulose fibers containing the butyl alcohol contain less than about 2 or 3% of water. Consequently, the water content of the mixed dope is of the order of 1%. There is no objection to carrying the dehydration below this point, but the solvent power of methyl alcohol for nitrocellulose rapidly falls off as the water content increases, so it is undesirable to exceed the percentages given.

While I have indicated a cylindrical wheel surface as a suitable one to carry the film-shaped dope when it passes through the setting bath, it will be understood that any of the well known forms of surfaces may be substituted, such as a belt having a polished even face.

Having thus described my invention, what I claim as new and desire to secure by Letters Patent is:

1. The process of making transparent,

flexible, nitrocellulose products of a form having great length relative to width and thickness, which comprises the steps of imparting such form to a solution of nitrocellulose in methyl alcohol containing a monohydroxy aliphatic alcohol of low volatility which is at least partially soluble in water, and treating it while in said form with an aqueous setting bath.

2. The process of making transparent, flexible, nitrocellulose products of a form having great length relative to width and thickness, which comprises the steps of imparting such form to a solution of nitrocellulose containing an excess of methyl alcohol and a monohydroxy aliphatic alcohol of low volatility which is at least partially soluble in water, removing said excess while it is in said form by treatment with a setting bath, which is a solvent of methyl alcohol and a non-solvent of nitrocellulose, removing the set product from said bath and drying the same.

3. The process of making transparent, flexible, nitrocellulose products of a form having great length relative to width and thickness, which comprises the steps of imparting such form to a solution of nitrocellulose in methyl alcohol containing normal butyl alcohol, and treating it while in said form with an aqueous setting bath containing methyl alcohol.

4. A process of making transparent, flexible, nitrocellulose film, which comprises the steps of imparting a film-form to a flowable solution of nitrocellulose in methyl alcohol containing from 30 to 100 parts by weight of a monohydroxy aliphatic alcohol of low volatility which is at least partially soluble in water, to 100 parts of nitrocellulose and treating it while in said form with an aqueous setting bath containing methyl alcohol, and stopping said treatment while a residuum of said alcohol of low volatility remains in said film.

5. The process of making transparent, flexible, nitrocellulose film, which comprises the steps of imparting a film-form to a solution containing 100 parts of nitrocellulose, 30 to 100 parts by weight of normal butyl alcohol, and 300 to 1000 parts by weight of methyl alcohol, and treating it while in said form with an aqueous setting bath containing at least 50% of methyl alcohol.

6. The process of making transparent, flexible, nitrocellulose products of a form having great length relative to width and thickness, which comprises the steps of imparting such form to a solution of nitrocellulose in methyl alcohol containing normal butyl alcohol and treating it while in said form with an aqueous setting bath containing methyl alcohol and normal butyl alcohol.

7. The process of making transparent, flexible, nitrocellulose film, which comprises the steps of forming on a polished surface a layer

70

80

85

90

95

100

105

110

115

120

125

130

of nitrocellulose dope containing methyl alcohol and a monohydroxy aliphatic alcohol of low volatility which is at least partially soluble in water, equalizing the thickness of 5 said layer on said surface, treating said equalized layer while on said surface, with a setting bath containing a liquid which is miscible with methyl alcohol but a non-solvent of nitrocellulose, and an amount of methyl alcohol insufficient to prevent setting of said layer, and removing from said surface the film thus prepared.

8. The process of making transparent, flexible, nitrocellulose film, which comprises the 15 steps of forming on a polished metallic surface a clear viscous layer of nitrocellulose dissolved in a mixture of methyl and normal butyl alcohols, allowing said layer to settle to lessen inequalities of thickness, treating 20 the equalized layer, while on said surface, with an aqueous setting bath containing an amount of methyl alcohol to prolong the setting action without stopping it, and removing from said surface the film thus prepared.

25 9. The process of making transparent, flexible, nitrocellulose films, which comprises the steps of forming into film-shape a nitrocellulose dope in which the nitrocellulose is dissolved in a mixture of methyl alcohol and a 30 monohydroxy aliphatic alcohol of low volatility which is at least partially soluble in water, and treating it while in said shape to an aqueous setting bath containing a nitrocellulose solvent, the proportion of the latter 35 being decreased as the setting proceeds.

10. The process of making transparent, flexible, nitrocellulose films which comprises the steps of forming on a polished surface a clear viscous layer of nitrocellulose dissolved 40 in a mixture of methyl and normal butyl alcohols, moving said layer and an aqueous setting bath containing methyl alcohol relative to each other while the layer remains on said surface and in contact with said bath, 45 the latter being lowest in water content at the start of said relative movement and highest at the end thereof.

Signed at Rochester, New York this 8th day of February, 1928.

50 JACKSON B. WELLS.